

June 26, 1951

P. W. BRIDGMAN

2,558,035

METHOD AND APPARATUS FOR COLD DRAWING

Filed July 5, 1947

2 Sheets-Sheet 1



INVENTOR  
PERCY W. BRIDGMAN  
BY  
*D.C. Harrison*  
ATTORNEY

June 26, 1951

P. W. BRIDGMAN

2,558,035

METHOD AND APPARATUS FOR COLD DRAWING

Filed July 5, 1947

2 Sheets-Sheet 2



Fig. 3.



Fig. 4.

INVENTOR  
PERCY W. BRIDGMAN  
BY  
*D. C. Harrison*  
ATTORNEY

## UNITED STATES PATENT OFFICE

2,558,035

METHOD AND APPARATUS FOR COLD  
DRAWING

Percy W. Bridgman, Cambridge, Mass.

Application July 5, 1947, Serial No. 759,185

12 Claims. (Cl. 205—3)

1

This invention relates to the technique of extrusion and more particularly to a novel method and apparatus for cold drawing metals, alloys and other plastic materials.

It has been well established by experiment that many metals and other plastic materials have greatly increased capacity for deformation without fracture if they are deformed while subjected to high hydrostatic pressure. For example, tension specimens of ordinary steel pulled while under a hydrostatic pressure of about 400,000 p. s. i. elongated up to 300 fold (the reduction in area being 99.7%) before fracture, whereas similar specimens pulled at atmospheric pressure broke at elongations of less than two fold.

In view of the increased ductility imparted to metal by high pressure, it would appear that cold metal could be extruded through the die of a conventional extrusion press upon the application of sufficient pressure directly to the metal. However, such a procedure fails in practice, because the friction between the cold metal and the walls of the die is so great that the die will split before the pressure can be increased sufficiently to start extrusion.

In my copending application, Serial No. 668,654, a method was described wherein a solid plastic material such as a metal or alloy, is extruded by subjecting such material uniformly to a high hydrostatic pressure, thereby increasing its ductility and forcing the material, while in an increased state of ductility, through a die. In each of several modifications described therein, the body being extruded is subjected to high hydrostatic pressure on one side of the die and to atmospheric pressure on the other side. As a result, the body is under great axial compressive stress during its passage through the die and tends to deform laterally against the inner walls thereof, thus creating great frictional forces in opposition to the forces promoting the extrusion process. It was disclosed therein that the hydrostatic pressure required to produce a given reduction of area could be considerably reduced by combining the extrusion process with a drawing operation wherein a pulling force is exerted on the issuing metal. This has the disadvantage, however, that a large part of the material subjected to tension is no longer under the influence of the hydrostatic forces that confer improved ductility. Consequently, brittle materials, ordinarily capable of being extruded by hydrostatic pressure alone, frequently fail by tension in the combined process.

It is the primary object of the present inven-

2

tion to provide a method and apparatus for drawing a solid plastic material such as a metal or alloy through a die while under high hydrostatic pressure and in a greatly increased state of ductility. Another object of the invention is to provide a relief valve that is readily operable under high hydrostatic pressure. A still further object is to provide a simple method of firmly securing the reduced end portion of a body to be extruded to a guide member capable of exerting a high tensile force when hydrostatic pressure is applied to the surrounding fluid.

In general, the method of the present invention comprises passing a reduced portion of a body of solid plastic material through a die, subjecting the portions of said body on both sides of said die to high hydrostatic pressure and applying tension to said reduced portion of said body, for example by causing said pressure to force an extended portion of said reduced portion through an orifice.

The invention is further described with reference to the accompanying drawings, in which

Fig. 1 is an elevation, in diagrammatic cross-section, of a hydrostatic drawing apparatus in accordance with the invention;

Fig. 2 is an enlarged perspective view, with a portion broken out, of the pull rod 28 of Fig. 1;

Fig. 3 is an elevation, in diagrammatic cross-section, of a modified form of the apparatus shown in Fig. 1;

Fig. 4 is a sectional view taken along the line 4—4 of Fig. 3;

Fig. 5 is an elevation, in diagrammatic cross-section, of a preferred form of relief valve for use in the hydrostatic drawing apparatus of the invention.

As shown in Fig. 1, the apparatus of the invention comprises a hydraulic cylinder B having three chambers adapted to hold a liquid or other suitable medium M under high pressure, and a relief valve 12. The upper chamber 13 is equipped with a plunger 14 for applying pressure to the medium M and is separated from the intermediate chamber 15 by the drawing die 16 which is supported by a shoulder 17 in the cylinder B. The intermediate chamber 15, in turn, is separated from the lower chamber 18 by the extrusion plate 19, which has an orifice 20 and is supported on a shoulder 21. The relief valve 12 connected to the lower end of the hydraulic cylinder B may be of any suitable design, but in view of the high pressures used is preferably constructed in the novel manner described in connection with Fig. 5. In order to prevent leak-

age with the high pressures required in the medium M it is desirable that the forward end 22 of the plunger 14 is slideably fitted to the main portion thereof to provide space for compressible packing rings 23 that are forced outwardly against the cylinder walls under the influence of endwise pressure. For the same reason, packing rings 24 should be used at the seat of the threaded joint connecting the relief valve 12 to the cylinder B. The packing rings may be of lead or other suitable material. Lead packing rings have been found to be particularly effective in maintaining pressures of 200,000 p. s. i. and higher.

It is not necessary that the medium M, employed in the drawing operation, be a liquid. In fact, at the pressures employed, it is most probable that oil, for example, is congealed into a soft solid. It is necessary, however, that a solid medium be notably softer than the material to be extruded and soft enough to transmit approximately hydrostatic pressure, i. e. it must support only a relatively small shearing stress. An advantage obtained by using a soft solid rather than a true liquid is that possible leakage of the medium around the die and piston may be more effectively prevented.

To assemble the apparatus for use, an end portion 25 of the metal body 26 to be drawn is reduced in cross-section, as by machining or grinding, over a sufficient length to allow it to be passed through the die 16 and inserted in the closely fitting axial hole 27 in one end of the pull rod 28 which extends into the loosely fitting orifice 20 in the extrusion plate 19. With the novel design of the recessed end of the pull rod 28, the hydrostatic pressure exerted by the surrounding medium serves to join the pull rod securely to the reduced end portion of the body inserted in the recessed end thereof provided only that the edge of the joint is sealed air-tight by a non-porous sealing material such as soft solder 29. Referring to Fig. 2, a portion of the wall thickness of the axial hole 27 in the pull rod 28 is reduced to a few thousandths of an inch, for example by forming two diametrically opposite flattened portions 30 that extend along the outer surface of the pull rod for a length substantially equal to the depth of the hole. When the edge of the joint is sealed the application of hydrostatic pressure on the outer portion of the pull rod causes the thick portions of the walls to be forced inwardly with great pressure against the rod, while the flattened portions of the walls, being considerably thinner, readily give way by buckling. By making the axial hole 27 deep enough, an extremely large gripping force may be obtained. The forward end of the pull rod preferably is rounded to permit easy entrance thereof into passage 20 of Fig. 1.

With the apparatus assembled as shown in Fig. 1, pressure may be applied to the medium M within the cylinder B by exerting a downward force upon the plunger 14. The equalization of pressure between the upper chamber 13 and the intermediate chamber 15 takes place almost instantaneously through suitable passages 31 preferably disposed concentrically about the orifice of the die 16. By means of these passages the upper and intermediate chambers are so interconnected as to form a unitary drawing chamber subjecting both the entering and emerging portions of the body to a high hydrostatic pressure. The transmission of fluid pressure from the intermediate chamber 15 to the lower chamber 18,

however, is purposely retarded by providing only a minimum amount of clearance between the pull rod 28 and the orifice 20. When the desired high hydrostatic pressure has become equalized in all three chambers, the relief valve 12 is quickly opened, allowing medium M to escape from the lower chamber 18 at a much greater rate than it can enter through the clearance between the pull rod 28 and the orifice 20. The resulting great difference in pressure between the intermediate chamber 15 and the lower chamber 18 drives the pull rod 28 through the orifice 20 and thereby simultaneously draws the metal body 26 through the die 16. With proper coordination of the relief valve opening, the pull rod clearance, and the force applied to the plunger, the portions of the body entering and leaving the die are subjected to high hydrostatic pressure and are therefore in an improved state of ductility. Furthermore, under such conditions of coordination, the drawing process may be continued uninterruptedly until the lower end of the pull rod 28 reaches the end of its travel, for example as shown by the broken line in Fig. 1.

The use of a pull rod 28 is not essential to the operation of the apparatus, as the mechanically reduced portion of the body itself may be made of sufficient length to extend into the orifice 20, which need be only slightly larger in diameter than the throat of the die 16. In this case the extrusion plate 19 may be positioned quite close to the die 16, allowing only enough space between these members for the unrestricted flow of the oil or other medium from the passages 31 through the small clearance space between the reduced portion 25 of the metal body and the walls of the orifice 20.

It is sometimes difficult to provide an amount of clearance between the pull rod 28 and the walls of the orifice 20 sufficient for easy insertion of the pull rod, yet not so large as to cause an undesirable loss of medium from the upper chambers 13 and 15 under the high pressures used. This difficulty may be avoided by providing a minimum of clearance between the extrusion plate orifice and the pull rod and by employing means to keep the end of the pull rod away from the extrusion plate orifice until the pressure in all three chambers has been equalized. A modification of the apparatus of Fig. 1 employing these features is shown in Fig. 3. In this embodiment, the hydraulic cylinder C has an upper chamber 41 separated from a lower chamber 42 by an extrusion bushing 43 supported at its flanged end 44 on the shoulder 45. The die 46 is coaxially mounted in the base of a cup-shaped die holder 47 which has an outer cylindrical wall 48 slideably disposed within the cylinder C, and a coaxial inner cylindrical wall 49 which protrudes beyond the outer cylindrical wall 48. Passages 50 extend from the space between walls 48 and 49 to orifices lying within the confines of the diametrical dimension of an axially located recess 58 in the upper portion of the extrusion bushing 43. A collar 51 rests upon the shoulder 52 in the inner wall of the cylinder C and at least portions of said collar fit slideably around the protruding end of the inner wall 49. As shown in Fig. 4, passages for the flow of medium past the collar are provided by the spaces 53 between the slideably fitting portions 54. However, if the entire inner surface of the collar is made to fit slideably around the protruding end of the inner wall, other passage means, such as holes extending through the thickness of the collar

would be equally suitable. A liner 55 adapted to screw into the upper portion of the hydraulic cylinder C firmly clamps the collar 51 against the shoulder 52. A compression spring 56 acting between the collar 51 and the base of the die holder 47 is restrained from advancing the latter toward the extrusion bushing 44 by shear pins 57 extending from the slideably fitting portions 54 of the collar 52 into the protruding end of the inner wall 49. These shear pins extend from holes in the collar 51 to the holes in the inner wall 49, the holes being opposite each other when the spring 56 is sufficiently compressed to abut the edge of the outer wall 48 against the collar 51. The protruding end of the inner wall 49 extends sufficiently beyond the outer wall 48 to enable the plunger 68 to establish contact therewith and shear the guide pins during the early part of its stroke. A relief valve 59 is connected to the lower chamber 42 as in the previous modification.

A portion of the body 63 to be extruded is reduced in cross-section, as hereinbefore described, in order that it may be passed through the die orifice, but the reduced portion 62 is made of only such length that it or the end of an attached pull rod, is adjacent to but not within the orifice 61 of the extrusion bushing 43. With the relief valve 59 closed, sufficient force is applied to the plunger 68 to produce the desired hydrostatic pressure in the oil or other medium M contained within the cylinder C. By means of passages 50 and 61 this pressure immediately equalizes itself throughout the entire interior of the cylinder. While maintaining the force on the plunger, the relief valve 59 is opened to permit some of the medium M to escape from the cylinder as the plunger descends under constant application of force. In its descent, the plunger 68 makes contact with the protruding edge of the inner cylinder wall 49 of the die holder 47 and severs the shear pins 57. This allows the compression spring 56 to force the reduced end 62 of the metal body 63, or the end of a pull rod attached thereto, into the snugly fitting orifice 61, and brings the die holder 47 to rest against a blocking means comprising the upper surface of the flange 44 of the extrusion bushing 43. The end portion 62 of the body within the orifice 61 completely blocks the flow of oil from the upper portion of the apparatus into the lower chamber 42. A high hydrostatic pressure is thus maintained in the upper chamber 41 and in the recess 58 whereas the pressure in the lower chamber 42 continues to drop through escape of oil through the open relief valve 59. When the pressure difference becomes sufficiently great, the end portion 62 of the body is forced through the orifice 61 by hydrostatic extrusion. It is thus apparent that the body being drawn is subjected to high hydraulic pressure both before entering and upon emerging from the die, similarly as in the apparatus of Fig. 1.

With the high fluid pressures used, often ranging up to 250,000 p. s. i. and higher, ordinary high pressure valves have been found unsuitable, particularly where rapid opening of the valve is of primary importance. Thus, in the apparatus of Fig. 1 it is essential that relief valve 12 be adjusted from fully shut to fully open almost instantaneously, as otherwise a considerable amount of oil or other medium would pass through the clearance between the pull rod and the walls of the extrusion orifice before the pres-

sure in the lower chamber would drop sufficiently fast for the rod to begin extruding.

A preferred form of relief valve shown in Fig. 5 comprises a cylindrical housing H having an externally threaded reduced portion 71 adapted, for example, to cooperate with a threaded recess in the end of cylinders B or C in Figs. 1 or 3, respectively. An axial inlet passage 72 of small diameter extends from the outer surface of the reduced portion 71 to the apex of a conical valve seat 73, forming the base of a recess 74 axially disposed in the end wall of the pressure cylinder 15. An outlet passage 76 extends from the side wall of the recess 74, in the vicinity of the conical seat 73, to an external connection 77 on the housing H. Within the recess 74 is a loosely fitting closure member such as a hardened steel ball 78 adapted to effect a fluid-tight seal of the inlet passage 72 when the said ball is forced against the conical seat 73. Pressure against the ball is provided by contact with a boss 79 on the forward end 80 of a plunger acting within cylinder 15. In view of the high pressures used this plunger preferably consists of two slideably fitted parts 80 and 81 separated by a compressible packing 82 capable of being deformed outwardly against the cylinder walls under the influence of endwise pressure. The mouth of the pressure cylinder 15 is sealed by the cylinder head 83, which is seated against the shoulder 84. Fluid-tight seating of the cylinder head is assured by providing compressible packing 85 between the said cylinder head and the reduced portion 86 of the firmly tightened gland nut 87. The cylinder head 83 has a long stem 88 passing through an axial opening in the gland nut 87 and terminating in a threaded end adapted for connecting the axial passage 89 in the stem 88 with an auxiliary hydraulic pump.

In operating the relief valve for use in the drawing apparatus of the invention, fluid medium F under pressure supplied by an auxiliary pump drives the plunger within the cylinder 15 against the hardened ball 78, causing the latter to be forced against the conical seat 73. This effectively seals the inlet passage 72 and prevents the escape of fluid medium from the cylinder of the drawing apparatus. Since the cross-sectional area of the relief valve plunger is very much greater than the effective area of the hardened ball, a relatively small fluid pressure from an auxiliary pump is sufficient to seal the valve against the high pressure existing in the main cylinder of the drawing apparatus. To open the relief valve, pressure is removed from the plunger by releasing fluid medium F in any suitable manner. This permits the plunger and the hardened ball to descend under the influence of fluid pressure from the main cylinder, thus connecting passage 72 with the outlet passage 76 and thereby providing a path of escape for medium from the main apparatus cylinder.

One advantage of the relief valve described is that it possesses ease and rapidity of operation. Furthermore, there is no tendency for any of the moving parts to stick; and the fact that the closure member is forced straight against the seat without rotation is of particular advantage when using high pressures.

Metals and other materials, which cannot be successfully drawn at room temperature, may be hot drawn at much lower than normal temperatures by means of the method and apparatus of the invention. This modification requires

only the application of heat to the specimen to be drawn.

The increased ductility of a material under high hydrostatic pressure makes it possible in some instances to draw coiled rod through the die. Such rod straightens itself out in passing through the die and emerges in the same condition as if it had been straight initially. This feature is of considerable practical significance, since it permits an increased length of material to be drawn in a given size hydraulic chamber.

Due to the great increase in ductility, metals drawn under high hydrostatic pressure acquire a similarly great increase in strain hardening. The degree of strain hardening may be determined from the "flow stress," which is an increasing linear function of the natural strain (natural logarithm of the ratio of initial area to final area). Because of the great strains induced by drawing under hydrostatic pressure, it is possible to strain harden to flow stresses much greater than the maximum which can be attained by drawing the metal through reducing dies at atmospheric pressure without fracture.

While in this description specific examples of methods and means for carrying out the invention have been described in detail, these examples are given by way of illustration merely, and it is to be understood that the invention is not limited thereby but encompasses all methods and means within the scope of the appended claims.

What is claimed is:

1. An apparatus for drawing a body of solid plastic material through a die while under the influence of hydraulic pressure, comprising a first hydraulic chamber having at least one fixed end wall; a die coaxially disposed within said first chamber and having the emergent end thereof facing said end wall; passage means connecting portions of said first chamber adjacent said die; a coaxial passage in said end wall at least equal to the diameter of the throat of said die; a second hydraulic chamber communicating with said coaxial passage; medium within both chambers capable of transmitting hydraulic pressure; a relief valve connected to said second chamber; and means for applying pressure to said medium.

2. An apparatus according to claim 1, comprising a spring for urging said die toward said end wall; restraining means for said motion operable by said means for applying pressure to said medium; and blocking means for maintaining a space between said die and said end wall.

3. An apparatus according to claim 2, comprising a die coaxially mounted in the base of a cup-shaped member having an outer wall slidably disposed within said first hydraulic chamber, a coaxial inner wall having an end protruding beyond said outer wall, and passages interconnecting opposite faces of said base; a collar affixed to the inner wall of said hydraulic chamber; said collar having portions slidably surrounding the protruding end of said inner wall of the cup-shaped member and passages connecting portions of said cylinder on opposite sides of said collar; a compression spring between said collar and said base restrained by shear pins extending from said collar into said inner wall of said cup-shaped member; and a plunger in said hydraulic chamber capable of establishing contact with and moving said inner wall of the cup-shaped member to sever said shear pins.

4. An apparatus as claimed in claim 3, comprising a pull rod adapted to be secured to a reduced end portion of a body capable of passing through

said die, said pull rod having a larger diameter than the throat of said die and adapted to fit snugly within the coaxial passage in said end wall.

5. An apparatus according to claim 3, comprising a shoulder within said hydraulic cylinder to act as a support for said collar, and a liner adapted to fit within said cylinder, said liner having an externally threaded portion adapted to cooperate with an internally threaded portion of said cylinder to permit clamping said collar rigidly in place.

6. In an apparatus for drawing a body of solid plastic material through a die while the lateral surfaces of said body on each side of said die are subjected to hydrostatic pressure, a pull rod having an axial recess in one end thereof adapted to receive a reduced end portion of said body, said recess having a reduced wall thickness at one or more portions of the circumference capable of transmitting radial force to the body portion within said recess when the wall of said recess is subjected externally to said hydrostatic pressure.

25. 7. In an apparatus for drawing a body of solid plastic material through a die while the lateral surface portions of said body on each side of said die are subjected to hydrostatic pressure, a cylindrical pull rod having an axial recess in one end adapted to receive a diametrically reduced end portion of said body, the wall thickness of said pull rod being reduced in one or more places over a length substantially equal to the depth of said recess, whereby radial pressure is transmitted to the body portion within said recess when the wall of said recess is subjected to external hydrostatic pressure, and a rounded portion at the other end.

8. An apparatus for passing a body of solid plastic material through a die while under the influence of hydrostatic pressure, comprising a first hydraulic chamber having at least one fixed end wall; a die disposed within said first chamber and having the emergent end thereof facing said end wall; passage means connecting portions of said first chamber adjacent said die; a coaxial passage in said end wall at least equal to the diameter of the throat of said die; a second hydraulic chamber communicating with said coaxial passage; medium within both chambers capable of transmitting hydraulic pressure; means for applying pressure to said medium; and a relief valve comprising a housing having a valve chamber communicating with said second hydraulic chamber, said valve chamber having a valve seat and a lateral outlet passage and opening into a pressure chamber; a closure member adapted to cooperate with said valve seat to seal said inlet passage; a plunger comprising two slidably fitted coaxial members of substantially equal diameters separated by compressible packing material capable of being deformed outwardly against the inner walls of said pressure chamber, said plunger having a coaxial boss capable of entering said valve chamber and forcing said closure member against said seat; and fluid-tight passage means associated with said pressure chamber to actuate said plunger.

9. A method of drawing a body of solid plastic material through a die, which comprises reducing a portion of said body to a cross-section adapted to pass through the throat of said die, passing said reduced portion through the throat of said die, subjecting the lateral surfaces of said body extending on both sides of said die to a high hy-

drostatic pressure, and applying an axially directed force to said body capable of urging the unreduced portion of said body through said die.

10. A method of drawing a body of solid plastic material through a die, which comprises reducing a portion of said body to a cross-section adapted to pass through the throat of said die, passing said reduced portion through the throat of said die, and subjecting the lateral surfaces of said body extending on both sides of said die and a transverse surface adapted to transmit axial force to said body to a high hydrostatic pressure, said hydrostatic pressure acting against said transverse surface imparting a resultant axial force upon said body capable of urging the unreduced portion of said body through said die.

11. A method of drawing a body of solid plastic material through a die, which comprises reducing a portion of said body to a cross-section adapted to pass through the throat of said die, passing said reduced portion through the throat of said die, and subjecting the lateral surfaces of said body on both sides of said die and a transverse surface of the unreduced portion of said body to a high hydrostatic pressure, said hydrostatic pressure acting against said transverse surface imposing a resultant axial force upon said body capable of extruding the unreduced portion of said body through said die.

12. A method of drawing a body of solid plastic

material through a die, which comprises reducing a portion of said body to a cross-section adapted to pass through the throat of said die, passing said reduced portion through the throat of said die, affixing to said reduced portion a tension member of larger cross-section than the cross-section of said reduced portion, thereby providing a transverse surface adapted to transmit axial force to said body, and subjecting the lateral surfaces of said body extending on both sides of said die, and said transverse surface to a high hydrostatic pressure, said hydrostatic pressure acting against said transverse surface producing a resultant axial force upon said body capable of pulling the unreduced portion of said body through said die.

PERCY W. BRIDGMAN.

#### REFERENCES CITED

20 The following references are of record in the file of this patent:

#### UNITED STATES PATENTS

| Number     | Name      | Date          |
|------------|-----------|---------------|
| 28 524,504 | Robertson | Aug. 14, 1894 |
| 524,505    | Robertson | Aug. 14, 1894 |
| 524,506    | Robertson | Aug. 14, 1894 |
| 524,508    | Robertson | Aug. 14, 1894 |
| 1,767,038  | Anderson  | June 24, 1930 |
| 1,777,611  | Grohek    | Oct. 7, 1930  |